

# UNITED STATES PATENT OFFICE.

CHARLES AUGUSTE PAILLARD, OF GENEVA, SWITZERLAND.

## METALLIC ALLOY.

SPECIFICATION forming part of Letters Patent No. 367,158, dated July 26, 1887.

Application filed March 6, 1886. Serial No. 194,325. (No specimens.) Patented in England May 11, 1886, No. 6,367, and in France May 11, 1886, No. 176,053.

*To all whom it may concern:*

Be it known that I, CHARLES AUGUSTE PAILLARD, of the city of Geneva, Switzerland, have invented a new and useful Improvement in the Manufacture of Spiral Springs for Watches and other Time-Pieces, (on which patents have been granted in England, No. 6,367, dated May 11, 1886, and France, No. 176,053, dated May 11, 1886,) of which the following is a full, clear, and exact description.

In spiral or hair springs for watches and other time-pieces it is very desirable to substitute for steel, of which they are usually composed, a substance which is neither oxidizable nor magnetic, but which shall possess some of the properties of steel—that is to say, small capabilities of dilatation, hardness, and elasticity.

My invention relates to a metallic alloy, and is composed of the metals hereinafter mentioned, or their equivalents, and is useful in the mechanic arts, and especially in the manufacture of balances, hair-springs, and the other parts of watch, clock, and chronometer mechanisms.

One object of my invention is to produce an alloy which shall be unoxidizable and non-magnetic.

A further object of my invention is to produce an alloy which shall possess some of the characteristics and properties of iron or steel—viz., hardness, elasticity, and ductility—and at the same time be substantially, if not absolutely, non-dilatable.

Many alloys have been made and used possessing some of the characteristics and properties above mentioned; but, so far as I know, no alloy has heretofore been made or used possessing all of the characteristics and properties possessed by the alloy hereinafter described and claimed.

In the manufacture of watches it is desirable, if not absolutely essential, that the balances and springs, and particularly the hair-springs, should be so constructed and be made of such metal that they will not rust or corrode, that they will not be affected by ordinary temperatures, nor by magnetic or electrical influences.

Numerous attempts have been made to produce balances and springs for watches which

will not be affected by any or all of the influences above mentioned, but, so far as I know, with only partial results. The failure to produce such springs and balances has been due in part to their construction, but principally and materially to the fact that a metal or alloy had not been found or used which would not be affected by any of the influences which interfere with and disturb the regularity and uniformity of their action.

The difficulties formerly experienced in producing balances and springs for watches which would resist the disturbing influences to which they were subjected have latterly been greatly augmented by the invention, production, and use of magnetic and electric machines and devices, possessing in some instances great magnetic and electrical attraction and force, which necessarily affect and disturb to a greater or less extent the regularity and uniformity of the action of such springs and balances of watches as are used and carried by persons operating and using, or who come within near proximity to, such machines and devices.

All of the difficulties mentioned, as well as those experienced by change of climate, season, locality, whether on land or sea, or either, of altitudes, the descent into mines of whatever character or depth, or from any cause or influence other than mechanical displacement or destruction, are practically, if not entirely, overcome by springs or balances properly made of the alloy invented and manufactured by me, forming the subject of this application.

My alloy is composed of palladium, copper, and iron, in about the following proportions, viz: Palladium, sixty to seventy-five parts; copper, fifteen to twenty-five parts; iron, one to five parts; but said proportions or percentages may be somewhat varied without changing or affecting the essential characteristics or properties of the alloy to any appreciable extent.

It is well known that palladium melts only at a very high degree of temperature, and for that reason I prefer to follow the process hereinafter described in forming this alloy, although other processes may be used.

In forming the alloy I take about one-half of the palladium to be used and put the same,

with the other metals to be used, in a clay crucible, adding thereto a small quantity of borax and powdered charcoal, and subject the same to heat until all of said metals are melted. I then add the remaining one-half part of the palladium to the molten mass, still subjecting the same to a high degree of heat until all of the palladium is melted. I then pour the entire molten mass into any suitable mold, and 10 when it is cooled it is ready for use.

I am aware that alloys have been made wherein palladium has been used and formed a component part of the alloy, as set forth in well-known publications and treatises on metals and their alloys. Such alloys, however, I do not broadly claim as my invention; but do claim, broadly, the alloy herein specified in about the proportions mentioned. In the manufacture of my alloy, composed of palladium, copper, and iron, I obtain a non-magnetic and unoxidizable product which has the properties of hardness, elasticity, and ductility,

and at the same time substantially, if not absolutely, non-dilatable. All of these properties have not heretofore been obtainable in a single alloy of this class, and by the use of the metals and their stated proportions, as set forth herein, an alloy is formed which possesses all of the named properties, and which is useful in the mechanical arts. 30

Having thus described my invention, what I claim, and desire to secure by Letters Patent, is—

1. An alloy composed of palladium, copper, and iron in about the proportions specified. 35
2. An alloy composed of palladium, sixty to seventy-five parts; copper, fifteen to twenty-five parts; and iron, one to five parts, substantially as described.

CHARLES AUGUSTE PAILLARD.

Witnesses:

CHARLES WILLIS WARD,

WILHELMINA STRUSS.